

## UNITED STATES PATENT OFFICE

EDWARD J. MAGUIRE, OF BROOKLYN, NEW YORK, ASSIGNOR TO THE GRASSELLI CHEMICAL COMPANY, OF CLEVELAND, OHIO, A CORPORATION OF DELAWARE

## PROCESS OF PREPARING ANIMAL SKINS FOR TANNING

No Drawing.

Application filed January 24, 1930. Serial No. 423,263.

Animal skins or hides are before tanning submitted to a number of treatments, which, among others, are intended to remove from the skins and hides such substances or flesh tissues which would interfere with the production of leather.

All skins contain substantial amounts of natural greases and fats, which, particularly in the case of sheep skins are not removed 10 in the dehairing, liming, bating, etc. operations, and such skins are before tanning usually submitted to a special degreasing process. The common degreasing processes consist in treatments with organic fat solvents, such as naptha, carbon-tetrachloride 15 and kerosene oil or others.

I have found that the natural greases and fats associated with animal skins can be removed by treating the skins with an aqueous 20 solution of tri-sodium phosphate. The greases and fats are emulsified or otherwise dissolved in the aqueous solution and are in this manner removed from the skins. It is possible to recover, as will be explained below, 25 the greases and fats, and particularly wool grease from the aqueous grease and fat emulsions or solutions obtained. My invention is particularly adapted to the treatment of any animal skin which after processing 30 requires the skin to be free of grease, such as the skins from sheep, goats, rabbits or other small animals.

The dehaired skins are easily and effectively degreased by means of an aqueous tri-sodium phosphate bath, which is applied to 35 the pickled skins direct, preliminary to tanning.

In performing the novel process of my invention I prepare an aqueous tri-sodium phosphate solution containing, for instance, 40 from about  $\frac{1}{2}$  to about 3% tri-sodium phosphate dodecahydrate or equivalent amounts of other hydrates. The skins are steeped therein for several hours at a temperature 45 ranging from about  $70^{\circ}$  to about  $110^{\circ}$  F. It will, of course, be understood by those skilled in the art that the use of higher temperature might injure the skins themselves. The skins are then taken out of the bath, if desired, 50 passed on to rollers to squeeze out the excess

solution, freely rinsed in water and are ready for subsequent processing. The equipment found in normal beam house practice, such as pits, paddle wheels, etc., can be conveniently used in my novel process. The special 55 apparatus designed for extracting the skins with organic solvents is also easily converted for application of my novel process, it being understood that no distillation and recovery of the solvent is required.

The tri-sodium phosphate treatment when applied to pickled skins depletes somewhat the skins and loosens the fibres, which is desirable in producing certain kinds of sheepskin leather, such as used for wearing apparel. This depleting effect of the tri-sodium phosphate on skins intended to be made into heavier leather can be corrected by a light sulfuric acid, sodium chloride pickle following the degreasing operation. The depleting 65 effect can, to a certain extent, be prevented or diminished by adding sodium chloride to the degreasing tri-sodium bath.

The spent tri-sodium phosphate solution is usually discarded, but if desired, the fats and 70 greases or soaps can be recovered as such, or in the form of fatty acids by acidifying the spent solution.

The amount of solution needed is conveniently figured at between  $\frac{1}{2}$  to 1 gallon per 75 20 pounds of hide. This is, of course, not critical. It is to a certain extent dependent upon the type of equipment used, the condition of the hides and other factors entirely independent of the principle of the action of 80 the tri-sodium phosphate. In a similar way the concentration of the solution, the temperature, and the duration of the action are interdependent and can be varied within very wide limits without departing from the spirit 85 of my invention. It will be understood that good agitation, increased temperature and increased concentration within the conditions limited by a maximum of about 3% tri-sodium phosphate concentration and about  $110^{\circ}$  90 F. will speed up the degreasing action. On the other hand concentrations below  $\frac{1}{2}\%$  can be used if sufficient solution is applied to the skins, and the solution be given ample time 95 to act. As a rule, the specific conditions un-

der which my novel process is applied will have to be adjusted to the practice of and equipment available at the particular factory where this process is adopted.

5 While it is not customary to degrease heavy, dehaired calf or steer hides before tanning, I found that my novel process is also applicable to this type of hides, and will remove such grease or fat associated therewith, 10 and in this manner avoid any treatment which might be necessary on the tanned leather if the dehaired skins had contained fats or greases. For this type of skins I use substantially the same concentrations, temperatures and other conditions as on sheep or other like, dehaired skins, but I prefer to add water soluble mineral salts to the tri-sodium phosphate bath to counteract the depleting or swelling action of the degreasing agent. 15 20 Common salt, Glauber's salt, Epsom salt, barium chloride and other similar substances were found convenient for this purpose. The concentration of these salts in the tri-sodium phosphate bath is not very critical and depends upon the plumping action desired. It can vary from a few per cent to saturation of the bath.

25 Tri-sodium phosphate in aqueous solution has a similar degreasing action on animal skins with hair or wool attached, and produces at the same time a loosening of the wool or hair. This loosening effect is, however, in most instances insufficient to allow of a practical removal of the hair and wool 30 and I prefer therefor to use other depilatories and degrease the skins with tri-sodium phosphate after they have been dehaired; which operation can be proceeded with at any stage before tanning.

35 40 The plumping action which tri-sodium phosphate shows on skins immersed in its aqueous solutions can also be made use of to soften or soak salted skins before they are submitted to depilation. A fraction of a 45 per cent of tri-sodium phosphate added to the soak produces in a very short time a soft, pliable stock which is in a very desirable condition for further treatments. The conditions in such a soaking operation are so mild 50 that very little degreasing takes place and the skins soaked in a very light tri-sodium phosphate will have to be submitted to a special degreasing operation after dehairing.

I claim:

- 55 1. In a process of preparing animal skins for tanning the step of steeping said skins in an aqueous solution of tri-sodium phosphate.
2. In a process of preparing animal skins for tanning the step of steeping the dehaired 60 skins in an aqueous solution of tri-sodium phosphate.
3. In a process of preparing animal skins for tanning the step of steeping the dehaired skins in an aqueous bath containing tri-sodium phosphate in an amount equivalent to

from about  $\frac{1}{2}$  to about 3% of the weight of the bath of tri-sodium phosphate dodecahydrate.

4. In a process of preparing animal skins for tanning the step of steeping the dehaired skins at a temperature of from about 70 to about 110° F. in an aqueous bath containing tri-sodium phosphate in an amount equivalent to from about  $\frac{1}{2}$  to about 3% of the weight of the bath of tri-sodium phosphate 70 dodecahydrate. 75

5. The process of degreasing sheep skins which comprises steeping said skins before tanning in an aqueous tri-sodium phosphate bath. 80

6. In a process of preparing sheep skins for tanning the step of steeping the skins, freed from wool in an aqueous bath at about 70 to 110° F. containing tri-sodium phosphate in an amount equivalent to about  $\frac{1}{2}$  to 3% tri-sodium phosphate dodecahydrate. 85

7. In a process of preparing sheep skins for tanning the steps of steeping the skins freed from wool in an aqueous bath at about 70° to 110° F., containing tri-sodium phosphate in an amount equivalent to about  $\frac{1}{2}$  to 3% tri-sodium phosphate dodecahydrate, and, following this operation, giving the skins a slight pickle in a bath containing sulfuric acid and sodium chloride. 90 95

In testimony whereof, I affix my signature.

EDWARD J. MAGUIRE.

190

105

110

115

120

125

130